

## UNITED STATES PATENT OFFICE

2,311,080

## TEXTILE TREATMENT

Paul S. Pinkney, Wilmington, Del., assignor to  
E. I. du Pont de Nemours & Company, Wil-  
mington, Del., a corporation of Delaware

No Drawing. Application November 8, 1940,  
Serial No. 364,886

8 Claims. (Cl. 8—124)

This invention relates to the treatment with formaldehyde of textile materials which are reactive thereto. More particularly, it relates to a process for increasing the uniformity of reaction between formaldehyde and a textile material.

The term "textile material" is intended to include filaments, fibers, staple or yarns, whether in the finished stage or at some intermediate stage in the production thereof. The term also includes fabrics, whether knitted, woven or felted, as well as garments or other articles made from such fabrics.

It has long been known to react textile materials with formaldehyde. Such reaction has been carried out for the purpose of increasing the strength of textiles or to improve their resilience, crease resistance, crush resistance, crimp retention, resistance to shrinking, and to reduce the dry and wet elongation and the extent to which such materials are swelled by water.

Many of these previously known processes have been unsuccessful due to the non-uniformity of treatment or the embrittlement of the textile.

Processes used heretofore for treating textile materials with formaldehyde have involved treating the impregnated textile material in a hot-air chamber or on a drying cylinder. Treating on drying cylinders is applicable only to flat fabrics which are not too thick for efficient heating. Heating in a hot-air chamber is not satisfactory for yarn, rope, or staple, or for garments, because uniformity of treatment cannot be obtained unless heating is continued until all parts of the textile material have reacted to a maximum extent with the formaldehyde. This leads to extreme brittleness. When lower concentrations of formaldehyde are used, it is even more difficult to obtain uniformity of treatment due to the more marked effect of unevenness in the extent to which formaldehyde is lost by evaporation from the various portions of the textile material. When the heating period is reduced, the less exposed portions of the textile material are likely to be markedly undertreated.

It is, therefore, an object of the present invention to provide a process for reacting a textile material with formaldehyde with great uniformity and without objectionable embrittlement.

It is another object of the present invention to provide a process for uniformly reacting a textile material with the minimum quantity of formaldehyde to accomplish the desired effect.

Other objects of the invention will appear hereinafter.

The objects of this invention may be accomplished, in general, by impregnating a formaldehyde-reactive textile material with the desired quantity of an aqueous solution of formaldehyde together with an acid-reacting catalyst, drying the impregnated material and heating the same to the desired reaction temperature by immersing the same in a hot, substantially anhydrous liquid which is substantially inert to water; i. e., which is not hydrolyzable.

The following examples illustrate in great detail the preferred methods of carrying out the process of this invention. It is to be understood, however, that the present invention is not limited to the specific details set forth therein.

## EXAMPLE I

20 Skeins of 150-denier, 40-filament, 2.8-turns per inch twist, bright unfinished viscose rayon yarn are impregnated with a water solution containing the amounts of formaldehyde and ammonium chloride indicated in Table I. The saturated skeins are centrifuged to remove excess solution, and immersed in boiling benzene for 1 hour. Water is distilled with the benzene during this heating step so that the yarn is, in effect, dried and then heated under substantially anhydrous conditions. The skeins are centrifuged, dried at room temperature, treated with a 1% aqueous ammonium hydroxide solution at 50° C. for 5 minutes, rinsed, and dried. Results of this treatment are summarized in Table I:

Table I

|            | Formaldehyde | Ammonium chloride | Crease angle | Increase in wet strength | Decrease in elongation |          |
|------------|--------------|-------------------|--------------|--------------------------|------------------------|----------|
|            |              |                   |              |                          | Wet                    | Dry      |
| 40         | Per cent     | Per cent          | Degrees      | Per cent                 | Per cent               | Per cent |
| Control... | None         | None              | 90           | —                        | —                      | —        |
| A.....     | 13           | 0.4               | 143          | 3                        | 76                     | 71       |
| B.....     | 8            | 0.25              | 122          | 25                       | 56                     | 58       |
| C.....     | 4            | 0.12              | 99           | 13                       | 8                      | 7        |

When the treated yarns are dyed with du Pont "Pontamine" Sky Blue 6BX (Rowe Color Index No. 518), a direct cotton dye, it is very apparent 50 that the yarn in each skein is uniformly modified throughout the skein. The affinity of viscose rayon for direct cotton dyes is lowered by treatment with formaldehyde to an extent which varies with the severity of the treatment. Thus, when 55 part of a skein is more heavily treated with form-

aldehyde than the rest of the skein, it is dyed much lighter than the rest of the skein. Unevenness of this nature is very apparent when a skein of viscose rayon yarn is dyed after being treated with an aqueous solution containing 8% of formaldehyde and 0.25% of ammonium chloride, centrifuged, dried at 65°-70° C. for 2 hours, and baked at 150° C. for 3 minutes.

Crease angles of yarn of this type are determined by winding single threads over a double-edged knife blade under a tension of 50 grams, removing the tension after 15 minutes, cutting the thread along one edge of the knife, and determining the average angle of crease of about 10 of the resulting short lengths of thread after a relaxation period of 10 minutes. An increase in crease angle indicates improved resilience.

#### EXAMPLE II

A skein of viscose rayon yarn like that treated in Example I is impregnated with a water solution containing 3% of formaldehyde and 0.4% of ammonium chloride, centrifuged, dried at room temperature, immersed in xylene at 138° C. for 2 minutes, rinsed with methanol, treated for 3 minutes at 70° C. with a 1% aqueous ammonium hydroxide solution, washed for 3 minutes at 70° C. with a 0.25% soap-0.1% soda ash solution, rinsed, and dried.

The crease angle of the yarn is increased by this treatment from 90°—that of the untreated yarn—to 154°. Its wet strength is raised 5%, its wet elongation reduced 80%, and its dry elongation reduced 65%. Examination of the skein after dyeing with a direct cotton dye shows the treatment is quite uniform.

#### EXAMPLE III

A skein of viscose rayon yarn like that treated in Example I is impregnated with a water solution containing 3% of formaldehyde and 0.4% of ammonium chloride, centrifuged, and dried at room temperature. It is immersed for 2 minutes in bis(methoxyethoxyethyl) ether at a temperature of 138° C. The treated yarn shows uniformly improved resilience. Butoxyethoxyethyl acetate can be used as the liquid heating medium with the same advantageous results.

#### EXAMPLE IV

There are described in U. S. application Serial No. 318,326, filed February 10, 1940, by William D. Nicoll, new high tenacity crimped regenerated cellulose filaments and fibers and a process for producing them which comprises the steps of spinning filaments from a viscose solution into a single coagulating and regenerating bath and relaxing the filaments, free from tension, in an aqueous liquid, said steps being carried out in accordance with certain critical relationship factors listed in the application. A skein of yarn prepared by this process is impregnated with a water solution containing 3% of formaldehyde and 0.4% of ammonium chloride, centrifuged, and dried at room temperature. It is immersed for 1 minute in xylene heated to 138° C. and washed according to the procedure used in Example II. The crease angle of the yarn is increased by this treatment from 86°—that of the untreated yarn—to 133°; its wet strength is increased 14%; and its elongation, both dry and wet, is lowered. The treated yarn shows uniformly improved crimp retentivity and resistance to swelling by water. Non-uniform modification of a skein of this yarn treated simi-

larly except that it is heated in air is quite apparent when the yarn is dyed.

#### EXAMPLE V

5 High tenacity viscose rayon yarn prepared by the process described in U. S. Patents Nos. 2,083,252 and 2,133,714 is wound on a bobbin, impregnated with a water solution containing 5% of formaldehyde and 0.5% of ammonium chloride, centrifuged, and dried at room temperature. It is immersed for 30 seconds in boiling xylene, rinsed with benzene, dried, washed with a warm 1% aqueous ammonium hydroxide solution, rinsed, and dried. The improved resilience of the 10 yarn treated in this manner is shown by the rise in crease angle from 113°—that of the untreated yarn—to 133°. The treated yarn shows lowered elongation and improved resistance to swelling by water. Yarn of this type treated similarly except that it is heated in air is markedly less uniformly modified.

#### EXAMPLE VI

25 Skeins of the new crimped viscose rayon yarn 2,500-denier, 100-filament, 2-turns per inch twist) described and claimed in U. S. application Serial No. 180,976, filed December 21, 1937, by William Hale Charch and William Frederick Underwood, are treated according to the procedure of 30 Example I. This new yarn is produced as described and claimed in the above application by the extrusion of viscose into a coagulating bath having a rapid coagulating action and a slow, or no, regenerating action with a velocity of extrusion at least 4 times the velocity of draw-off. The streams of viscose issuing from the spinneret into the coagulating bath under the aforementioned conditions spontaneously assume a finely crimped 35 form which persists as a permanent structural characteristic in the filaments. The resulting yarn is composed of substantially non-crenulated filaments having an inherent and substantially permanent crimp, the crimps in the several filaments of the yarn being out of phase with each other. The filaments exhibit substantially no 40 orientation in the direction of the fiber axis.

45 Results of the formaldehyde treatment are summarized in Table II. The figures given in the table to represent the changes in properties effected by the treatment are, of course, with reference to untreated yarns.

Table II

| 55 | Formaldehyde | Ammo-nium chloride | Crease angle | Increase in wet strength | Decrease in elongation | Decrease in spontaneous extension when wet | Decrease in secondary swelling |
|----|--------------|--------------------|--------------|--------------------------|------------------------|--------------------------------------------|--------------------------------|
| 60 | Con-trol     | Per cent           | Per cent     | Degrees                  | Per cent               | Per cent                                   | Per cent                       |
|    | A            | None               | 0.4          | 66                       | 135                    | 65                                         | 100                            |
|    | B            | 8                  | 0.25         | 129                      | 144                    | 37                                         | 63                             |
|    | C            | 4                  | 0.12         | 76                       | 47                     | 42                                         | 46                             |

65 Crease angle measurements on the yarn are made in much the same manner as described in Example I except that the length of yarn to be tested is hung from a double-edged knife with a 500-gram weight for 2 minutes, wound around the blade, and cut along one edge after 10 minutes. The angles are let relax for 10 minutes before measuring.

70 Secondary swelling is measured by wetting 75 weighed skeins of untreated and treated yarns

with water, centrifuging them together, and weighing each in a closed container to determine the amount of water retained. The untreated yarn usually retains a quantity of water approximately equal to the weight of the yarn. The secondary swelling of treated yarn is expressed as per cent relative to that of the untreated yarn. This untreated yarn extends spontaneously when wet with water until it is 40%–50% longer than when dry.

The excellent uniformity of treatment by the process of the present invention is apparent upon examination of skeins of the treated yarn after dyeing with a direct cotton dye. On the other hand the same yarn, when treated with a water solution containing 8% of formaldehyde and 0.25% of ammonium chloride, centrifuged, dried at 65°–75° C. for 2 hours, baked at 153° C. for 3 minutes in an oven, and dyed with a direct cotton dye, is colored very unevenly. This unevenness indicates a very non-uniform treatment.

#### EXAMPLE VII

A skein of crimped viscose rayon yarn like that treated in Example VI is impregnated with a water solution containing 3% of formaldehyde and 0.4% of ammonium chloride, centrifuged, and immersed for 10 minutes in xylene heated to 138° C. The yarn is improved uniformly by this treatment in resilience and wet strength.

#### EXAMPLE VIII

Skeins of crimped viscose rayon yarn like that treated in Example VI are impregnated with water solutions containing 0.4% of ammonium chloride and the amounts of formaldehyde indicated in Table III, centrifuged, dried at room temperature, immersed for the indicated period of time in xylene heated to 138° C., and washed by the procedure of Example II. Results of the treatments are summarized in Table III. Dyeing tests show the treatments are all quite uniform.

When bis(ethoxyethyl) ether is used instead of xylene, the results are equally favorable. This solvent has the added advantage of being miscible with water and, therefore, readily removable from the fabric.

Table III

| Control | Formaldehyde | Time of immersion | Crease angle | Increase in wet strength | Decrease in elongation | Decrease in secondary swelling |
|---------|--------------|-------------------|--------------|--------------------------|------------------------|--------------------------------|
|         | Per cent     | Minutes           | Degrees      | Per cent                 | Per cent               | Per cent                       |
| Control | None         | 66                | 66           | 13                       | 32                     | 28                             |
| A       | 1            | 1                 | 70           | 15                       | 33                     | 44                             |
| B       | 1            | 2                 | 72           | 15                       | 33                     | 44                             |
| C       | 1            | 5                 | 87           | 35                       | 33                     | 62                             |
| D       | 2            | 2                 | 105          | 92                       | 58                     | 66                             |
| E       | 2            | 5                 | 108          | 72                       | 53                     | 80                             |
| F       | 3            | 1                 | 113          | 81                       | 48                     | 63                             |
| G       | 3            | 2                 | 123          | 110                      | 48                     | 77                             |
| H       | 3            | 5                 | 156          | 75                       | 61                     | 89                             |
| I       | 5            | 1                 | 166          | 84                       | 53                     | 82                             |
| J       | 5            | 2                 | 180          | 55                       | 58                     | 85                             |
| K       | 10           | 2                 | 180          | 0                        | 63                     | 85                             |

#### EXAMPLE IX

Gel staple fibers prepared by the process of U. S. application Serial No. 180,976, referred to in Example VI are impregnated with a water solution containing 2% of formaldehyde and 0.4% of ammonium chloride, centrifuged, and dried at room temperature. They are immersed for 5 minutes in mineral oil heated to 145° C. and then thoroughly washed with soap to remove the oil. The treated fibers show improved resilience and resistance to swelling in water. Dyeing tests show

the treatment is uniform throughout. Fibers in staple form are particularly difficult to heat uniformly in air.

#### EXAMPLE X

- 5 A rope of yarn of the type treated in Example VI is impregnated with a water solution containing 2% of formaldehyde and 0.2% of ammonium chloride, centrifuged, and dried at room temperature. It is immersed for 5 minutes in 10 triethanolamine heated to 150° C. and then washed with water. The treated fibers show uniformly improved resilience and resistance to swelling in water. Rope of this nature is too thick to be heated uniformly throughout in a 15 short time in air.

#### EXAMPLE XI

- Two skeins of crimped viscose rayon, like that treated in Example VI, are impregnated with a 20 water solution containing 0.4% of ammonium chloride and 1% and 3% of formaldehyde, respectively, centrifuged, and dried at room temperature. They are immersed for 1 minute in Wood's metal heated to 138° C., washed with an 25 alkaline soap solution, rinsed, and dried. Both treated skeins show uniformly improved resilience and resistance to swelling in water.

#### EXAMPLE XII

- 30 Transparent velvet having a viscose rayon pile and silk backing is impregnated with a water solution containing 13% of formaldehyde and 0.4% of ammonium chloride, centrifuged, and placed in 35 boiling benzene for 1 hour. It is then dried, rinsed with warm dilute ammonium hydroxide solution, and soaped for 1 minute at 70° C. with a 0.25% soap-0.1% soda ash solution. The resilience of the pile is improved by this treatment.

#### EXAMPLE XIII

- 35 Samples of transparent velvet having a viscose rayon pile and silk backing are impregnated with a water solution containing 0.4% of ammonium chloride and 2% and 5% of formaldehyde, respectively, centrifuged, and dried at room temperature. They are immersed for 1 minute in xylene heated to 138° C., rinsed with methanol and water, heated in dilute ammonium hydroxide solution at 70° C. for 3 minutes, and then in an 45 50 alkaline soap solution at 70° C. for 3 minutes, and rinsed. Both samples show improved resilience.

#### EXAMPLE XIV

- 55 A viscose rayon stocking is impregnated with a water solution containing 3% of formaldehyde, 0.3% of stearylamine hydrochloride, and 0.4% of ammonium chloride, centrifuged, dried at room temperature on a board, and immersed for 1 minute in xylene heated to 138° C. The stocking is then washed by the procedure of Example II 60 and dried on a board. The treated stocking shows improved hand and resistance to wrinkling and dries much more rapidly than an untreated control.

#### EXAMPLE XV

- Viscose rayon yarn spun from viscose containing casein as described in British Patent No. 501,531 is impregnated with a water solution containing 3% of formaldehyde and 0.4% of ammonium chloride, centrifuged, and dried at room temperature. It is immersed for 1 minute in xylene heated to 138° C. and then washed. The 70 treated yarn shows uniformly improved resilience and wet strength and lowered elongation.

As above set forth, if any formaldehyde-reactive textile material is impregnated with aqueous formaldehyde and an acid-reacting catalyst, dried and then heated by immersion in a hot substantially anhydrous liquid which is substantially inert to water under the conditions prevailing during the heating step, an improved and more uniformly treated product will be obtained.

As a "formaldehyde-reactive textile material", the present invention contemplates the treatment of filaments, yarns, fabrics and the like comprising regenerated cellulose, regenerated protein materials, and low substituted cellulose esters and ethers; i. e., cellulose esters and ethers having at least one unsubstituted hydroxyl group.

The present invention is operative in the treatment of all textile materials which are at all reactive to formaldehyde. In the treatment of such textiles as are less reactive than those specifically referred to above, the treating conditions will, of course, be more drastic.

The term "textile material" includes fibers in the form of loose staple, yarn, fabric, or finished article and filaments in the form of yarn, fabric, or finished article. The fabrics may be knitted, woven, or felted. They may be special types of fabric such as pile fabrics or crepe. Viscose rayon fibers may be treated in the gel state either as staple, rope, or yarn.

The term "acid-reacting catalyst" is intended to include water soluble substances which are acid in reaction, or capable of becoming acid under the conditions of the treatment, or capable of liberating an acid under the conditions of the treatment. Examples are organic carboxylic or sulfonic acids such as oxalic acid, tartaric acid, and benzenesulfonic acid, acid salts of organic acids such as sodium acid tartrate and potassium tetroxalate, mineral acids such as hydrochloric acid, sulfuric acid, and phosphoric acid, acid salts of mineral acids such as sodium bisulfate and dihydrogen sodium phosphate, and salts of strong acids with weak bases which dissociate in water solution to give an acid reaction such as ammonium thiocyanate, ammonium chloride, ammonium bromide, ammonium iodide, ammonium sulfate, hydroxylamine hydrochloride, ferric chloride, calcium chloride, aluminum chloride, etc. The catalyst chosen in any particular case will be the one which is sufficiently powerful to effect the degree of chemical reaction desired between the textile material and the formaldehyde. Because of its cheapness and effectiveness, ammonium chloride is the catalyst which is preferred in the exercise of this invention.

As liquids suitable for use as heating media in the process of this invention, there may be used any substantially anhydrous liquid boiling above 70° C. and preferably above 100° C. which is substantially inert to water under the conditions prevailing during the heating step. Examples are hydrocarbons such as benzene, toluene, xylene, kerosene, mineral oil, high boiling benzine, triisobutylene, etc., esters such as butyl acetate, tricresyl phosphate, dimethyl phthalate, "Cellulosolve" and Carbitol esters, butyl borate, etc., alcohols, such as glycerol, ethylene glycol, butanols, octanols, etc., halides such as tetrachlorooctane, tetrachloroethylene, chlorobenzene, bromobenzene, tribromoethane, amylene dichloride, chloronaphthalene, chlorotoluene, dichlorobenzenes, etc., hydroxy ethers such as

"Cellulosolves" and Carbitols, ethers such as diisobutyl ether, bis(methoxyethoxyethyl) ether, and dioxane, amines such as monoethanolamine, diethanolamine, triethanolamine, dimethylamine, etc., and low melting metals or alloys such as Wood's metal, Rose metal, and mercury. The organic liquids used may be aliphatic or aromatic, saturated or unsaturated. Of course, esters and ethers which are solvents for cellulose esters and ethers cannot be used as heating media in treating textile materials composed of the latter substances. In any case the liquid used should preferably be easily removed from the textile material, stable toward heat, inert toward water, non-toxic, and non-flammable. Bis(methoxyethoxyethyl) ether and bis(ethoxyethyl) ether are preferred heating liquids in carrying out the present invention.

The formaldehyde treating solution may contain desired modifying agents which will improve the resulting product, as long as the modifying agent does not interfere with the reaction between the formaldehyde and the textile material. For example, long chain agents such as glycerol monostearate or sulfonated castor oil may be added to the formaldehyde solution to improve hand and feel of the textile material. However, when such a long chain agent is used and the liquid heating medium used is a solvent for it, it is preferable to saturate the liquid heating medium with the long chain agent so that the agent will be retained by the textile material and not dissolved out by the heating medium.

The concentration of formaldehyde to be used in the treating solution varies, of course, with the material under treatment, the nature and concentration of the catalyst, the nature and concentration of modifying agents, the conditions of drying and heating, and the effect desired. For example, for creaseproofing viscose rayon a higher formaldehyde concentration is required than for shrinkproofing the material, other conditions remaining the same. Generally, when the drying and heating conditions are more severe, that is, when higher temperatures and longer times are employed, less formaldehyde is required. Thus, if the impregnated material is dried at 100° C. rather than at room temperature, less formaldehyde will be required to give the same final effect. Generally, to obtain comparable effects, less formaldehyde is required when a more strongly acidic catalyst is employed or when a catalyst is used in higher concentrations, than when a more weakly acidic catalyst is employed or when a catalyst is used in lower concentrations. Usually, a concentration of formaldehyde of at least 1% is required to obtain a noticeable effect on cellulosic materials. The upper limit is the concentration at which the particular textile material being treated is made too weak or too brittle for use. As a general rule, the formaldehyde concentration should not exceed 20%. With these facts in mind, one skilled in the art can readily determine the concentration of formaldehyde which will give optimum results under a given set of other conditions.

The catalyst concentration may vary from as low as 0.05% or lower to as high as 1% or higher depending on the potential acidity of the catalyst, the nature of the textile material under treatment, the concentration of formaldehyde employed, the nature and concentration of modifying agents, the drying and heating conditions,

and the effect desired. Other conditions remaining the same, an increase in the catalyst concentration or a change from a less to a more strongly acid catalyst results in a greater degree of modification of the textile material. Usually, the selection of the nature and concentration of the catalyst is a matter of balancing catalyst efficiency against tendering which results from the use of acidic materials on many textile materials, particularly cellulosic materials. By reference to the above examples and the following description one skilled in the art can readily select the proper catalyst and concentration to bring about the desired result.

The treating solution may be applied to the textile material in any of several ways. Staple fibers may be dipped in the solution and squeezed or centrifuged to remove excess solution. Yarn may be passed continuously through the solution or it may be dipped in skein form in the solution and then squeezed or centrifuged to remove excess solution. Flat fabrics may be passed through the solution or the solution may be applied from rolls or by spraying and the excess may be removed by squeezing between rolls or by 25 vacuum extracting. Articles, as of clothing, may be dipped in the solution or sprayed. Fabrics or articles of clothing may be treated locally by spraying.

The formaldehyde and catalyst may also be applied in other ways. For example, the textile material may be wet with a solution of the catalyst and then exposed to vapors of formaldehyde, or it may be wet with formaldehyde solution and then exposed to a gaseous catalyst such as hydrochloric acid.

After impregnation with the treating solution the textile material is preferably dried to a water content of about 15% or less before it is subjected to the final heat treatment. This may be carried out in any of several ways. It may be dried in air or in a heated inert liquid such as a hydrocarbon or ether. If it is air dried, the temperature of drying may range from room temperature to 150° C. or higher. Drying at high temperatures in air must be carried out with care so that no part of the textile material is heated after it is dry. Uniformity is favored by vigorous circulation of air in the drying chamber and by use of temperatures below 100° C., and preferably below 50° C. The most uniform drying, particularly for staple, large skeins of yarn, and garments, is obtained by use of a hot inert liquid in which water is preferably no more than slightly soluble. Liquid temperatures up to 250° C. or higher may be used. If a temperature below 100° C. is used, it is usually necessary to boil the drying liquid in order to carry out the water. Consequently, for drying at such temperatures liquids boiling below 100° C. are desirable. However, if they boil below about 70° C. the rate of drying will generally be too low for practical purposes.

The time of drying depends, of course, on the drying method used. When the air drying method is used, the time required depends on the temperature, circulation of air, and the relative thickness and looseness of the material under treatment. When the hot liquid drying method is used, the time required depends on the nature of the liquid and the temperature used and less on the construction of the material under treatment. In general, with temperatures below 100° C., the air drying method is more rapid and may require as short a time as 2 minutes. When the

material under treatment is in a relatively loose condition so that air will circulate through it freely, air drying has an advantage over drying in a hot liquid in that the formaldehyde concentration required for a given degree of modification is much lower and the overall period during which the material is held at the higher liquid temperature is shorter, so that the risk of tendering due to the effect of the acid reacting catalyst at high temperatures is less. At higher temperatures the liquid drying method is generally more rapid due to more efficient heat transfer between the moisture and the heating medium. If, for example, a liquid such as molten metal is used at a temperature in the range of from 200°-250° C. or higher, drying may be complete in a fraction of a second. In general, with other conditions remaining constant, an increase in the drying temperature leads to a greater degree of modification of the textile material.

In order to bring about a reaction between formaldehyde and the textile material within a reasonable time, it is necessary to heat the impregnated and dried material. In this process the heating step is carried out by immersing the textile material in a hot liquid of the nature disclosed above. The temperature of the liquid may be as low as 70° C. or lower, although a much longer heating period is required at such low temperatures. As already pointed out, if a heating temperature below 100° C. is used, that temperature should be the boiling point of the liquid so that water formed by the reaction will be removed efficiently. The temperature of the liquid may range as high as 200° C. or even higher. However, it should be emphasized that at such high temperatures the heating period should be reduced to the neighborhood of 1 second or less to avoid damaging the textile material. The heating temperature depends on the amount of formaldehyde used, the nature and amount of catalyst, the nature and amount of modifying agent, the temperature of drying, the time of heating, the effect desired, and the nature of the textile material under treatment. It is common knowledge that some textile materials are more susceptible to damage by heat than are others and so require more careful treatment in any heating process. In general, with other conditions remaining constant, an increase in the temperature of the heating liquid leads to a greater degree of modification of the textile material under treatment.

The heating period may be varied from as long as an hour or more at low temperatures, such as 55 70°-80° C. or lower, to a fraction of a second at higher temperatures, such as 200° C. or higher. When the heating is to be carried on over a period of about a minute or longer, it is advantageous to place the textile material in a perforated container which is lowered into the hot liquid bath and then lifted after the desired length of time. When yarn or fabric is to be heated at a higher temperature for a shorter period of time, it is advantageous to pass the yarn or fabric continuously through the heating bath at a rate depending on the length of bath travel. With other conditions remaining constant, an increase in the heating period leads to a greater degree of modification of the textile material under treatment.

From the above descriptions, it will be apparent that the drying step and the heating step may be combined into one continuous step. The drying liquid may be used for the subsequent heat

treatment. Thus, it is sometimes convenient to prolong the period of immersion in the drying liquid until the reaction between formaldehyde and the textile material has proceeded to the desired point.

After the heating step it is usually desirable to remove the heating liquid. This may be accomplished simply by evaporation of the liquid if the liquid is sufficiently volatile, benzene, for example. If the liquid is water soluble, triethanolamine, for example, it can be washed out with water. Water insoluble non-volatile materials may be displaced by a volatile or water soluble solvent or removed by soaping. It is usually desirable to neutralize any traces of acidic material which may be left in the yarn by washing with a solution of ammonium hydroxide or other mildly alkaline material. The treated material may then be finished in any desired manner such as by application of a softening agent or water repellent agent.

Since it is obvious that many changes and modifications can be made in the above-described details without departing from the nature and spirit of the present invention, it is to be understood that the invention is not to be limited to the said details except as set forth in the following claims.

I claim:

1. In a process for reacting a textile material with formaldehyde, the steps comprising impregnating said material with an aqueous solution of formaldehyde, drying said impregnated material, and heating the same to reaction temperature by immersion in an inert heating liquid at a temperature of between 70° C. and 200° C., whereby said material is uniformly reacted with the formaldehyde and objectionable embrittlement thereof is prevented.

2. In a process for reacting a textile material with formaldehyde, the steps comprising impregnating said material with an aqueous solution of formaldehyde and an acid reacting catalyst, drying said impregnated material, and heating the same to reaction temperature by immersion in an inert heating liquid at a temperature of between 70° C. and 200° C., whereby said material is uniformly reacted with the formaldehyde and objectionable embrittlement thereof is prevented.

3. In a process for reacting a regenerated cellulose textile material with formaldehyde, the steps comprising impregnating said material with an aqueous solution of formaldehyde, drying said impregnated material, and heating the same to reaction temperature by immersion in an inert

heating liquid at a temperature of between 70° C. and 200° C., whereby said material is uniformly reacted with the formaldehyde and objectionable embrittlement thereof is prevented.

4. In a process for reacting a regenerated cellulose textile material with formaldehyde, the steps comprising impregnating said material with an aqueous solution of formaldehyde and an acid reacting catalyst, drying said impregnated material, and heating the same to reaction temperature by immersion in an inert heating liquid at a temperature of between 70° C. and 200° C., whereby said material is uniformly reacted with the formaldehyde and objectionable embrittlement thereof is prevented.

5. In a process for reacting a regenerated cellulose textile material with formaldehyde, the steps comprising impregnating said material with an aqueous solution of formaldehyde, drying said impregnated material, and heating the same to reaction temperature by immersion in a liquid comprising a hydrocarbon, whereby said material is uniformly reacted with the formaldehyde and objectionable embrittlement thereof is prevented.

6. In a process for reacting a regenerated cellulose textile material with formaldehyde, the steps comprising impregnating said material with an aqueous solution of formaldehyde, drying said impregnated material, and heating the same to reaction temperature by immersion in a liquid comprising xylene, whereby said material is uniformly reacted with the formaldehyde and objectionable embrittlement thereof is prevented.

7. In a process for reacting a regenerated cellulose textile material with formaldehyde, the steps comprising impregnating said material with an aqueous solution of formaldehyde, drying said impregnated material, and heating the same to reaction temperature by immersion in a liquid comprising bis(ethoxyethyl) ether, whereby said material is uniformly reacted with the formaldehyde and objectionable embrittlement thereof is prevented.

8. The process of decreasing the secondary swelling of substantially non-crenulated and non-oriented, permanently crimped, regenerated cellulose filaments which comprises impregnating a textile material composed of said filaments with an aqueous solution of formaldehyde, drying said impregnated material, and heating the same to reaction temperature by immersion in an inert heating liquid at a temperature of between 70° C. and 200° C.

PAUL S. PINKNEY.